

No. 881,934.

PATENTED MAR. 17, 1908.

F. VON KÜGELGEN & G. O. SEWARD.

PROCESS OF PRODUCING ALUMINUM MAGNESIUM ALLOYS.

APPLICATION FILED APR. 27, 1905.



INVENTORS

WITNESSES:

Fred White  
Rene' Prune

Franz von Kugelgen & George O. Seward  
By Attorneys,  
William G. Fraser

# UNITED STATES PATENT OFFICE.

FRANZ VON KÜGELGEN AND GEORGE O. SEWARD, OF HOLCOMBS ROCK, VIRGINIA,  
ASSIGNORS TO VIRGINIA LABORATORY COMPANY, OF NEW YORK, N. Y., A COR-  
PORATION OF NEW YORK.

## PROCESS OF PRODUCING ALUMINUM-MAGNESIUM ALLOYS.

No. 881,934.

Specification of Letters Patent. Patented March 17, 1908.

Application filed April 27, 1905. Serial No. 257,618.

*To all whom it may concern:*

Be it known that we, FRANZ VON KÜGELGEN, a subject of the German Emperor, and GEORGE O. SEWARD, a citizen of the United States, both residing at Holcombs Rock, in the county of Bedford and State of Virginia, have jointly invented certain new and useful Improvements in the Process of Producing Aluminum-Magnesium Alloys, of which the following is a specification.

This invention relates to the production of alloys of aluminum and magnesium. Certain of these alloys have many valuable properties, and are in many respects more valuable than aluminum. They are easily cast, are lighter than aluminum, and are easily machined. Their melting point is low, and it is possible to make castings at a dull red heat. These alloys would supersede aluminum were it not for the high cost of the magnesium, and for the loss of magnesium when the metals are melted together to form the alloy.

Our present invention provides a process by which these alloys can be produced more cheaply than heretofore. Our process is characterized by the electrolytic decomposition of magnesium oxid dissolved in a suitable fluorid bath in the presence of a cathode of molten aluminum, or aluminum-magnesium alloy, with which the reduced magnesium alloys; or by the electrolysis of a combined bath of a magnesium compound and an aluminum compound, their reduced metals alloying at the cathode. The electrolytic bath is composed of magnesium oxid, or a mixture of aluminum oxid and magnesium oxid, dissolved in magnesium fluorid and a fluorid of a more electro-positive metal, the bath being of such specific gravity that the alloy produced remains at the bottom.

Our present invention is based upon our process for the production of magnesium characterized by the electrolytic decomposition of magnesium oxid dissolved in a molten bath of a metallic salt or salts; the best bath being of magnesium fluorid and a fluorid of a more electro-positive metal. We have discovered that this process is applicable to the production of aluminum-magnesium alloys by using a cathode of molten aluminum (or of such alloy) with which the separated magnesium alloys and remains

at the bottom of the electrolytic vessel. We have also found that aluminum oxid is easily dissolved in such a bath, and that aluminum-magnesium alloys are obtained when a mixture of aluminum oxid and magnesium oxid is fed to the fluorid bath instead of magnesium oxid alone.

Our process may be variously practiced, and the electrolytic cell or vessel may be variously constructed. We will describe in detail one suitable and preferable mode of practicing our process with reference to the accompanying drawing, which shows a suitable electrolytic cell for the purpose, the view being in vertical mid-section.

Referring to the drawing, let A designate a suitable vessel, such as an iron pot, which may have its sides cooled by a water jacket D. Such cooling would result in a chilled layer B of the electrolyte which would insulate the sides of the vessel so that no current would pass from the electrodes to the sides.

C is the molten metal cathode, which is at first of aluminum and subsequently of aluminum-magnesium alloy.

E is the molten electrolyte and F F the anodes of carbon or graphite. A dynamo or other generator G has its positive terminal connected to the anodes F F and its negative terminal to the pot A.

In practicing the process, a suitable quantity of aluminum is placed in the bottom of the vessel and the electrolyte is introduced and melted by the current. This electrolyte consists of magnesium oxid or magnesium oxychlorid dissolved in a suitable salt, preferably magnesium lithium fluorid. Or magnesium fluorid mixed with some other fluorid of a metal more electro-positive than magnesium may be used. The proportions of fluorid salts may greatly vary. The effect of the electrolysis is to decompose the dissolved magnesium oxid, the liberated magnesium going to the cathode where it alloys with the aluminum, so that the cathode becomes an aluminum-magnesium alloy where in the proportion of magnesium is continually increasing. When the desired proportion of magnesium is reached, the alloy is tapped out or otherwise removed from the vessel, and fresh aluminum is added. Magnesium oxid is fed continually into the electrolyte to replace that which is decomposed.

Instead of adding metallic aluminum, the

aluminum may be produced in the cell simultaneously with the magnesium by double electrolysis. To this end it is only necessary to mix aluminum oxid with the magnesium oxid and feed the mixed oxids into the fused bath instead of the magnesium oxid alone. Both oxids dissolve in the bath, and both are decomposed by the current, freeing both magnesium and aluminum at the cathode, so that the metals alloy continuously. By mixing the oxids in the proper proportions, the resulting alloy can be produced of any desired composition or richness. The process is thus rendered substantially a continuous one, it being only necessary to tap off the alloy from time to time without paying any attention to its composition.

Instead of using magnesium oxid, we may use magnesium oxychlorid, which is easily obtained free from water, is soluble in a fluorid bath, and is decomposed in the same way as magnesium oxid, except that both chlorine and oxygen are liberated at the anode. By the expression "magnesium oxid" in our claims, we desire it understood that magnesium oxychlorid is included, as well as any other magnesium compound of analogous composition and properties.

Our process produces the desired aluminum-magnesium alloys at low cost, and avoids the loss due to melting magnesium and aluminum together to form the alloy.

It is not to be understood from the particularity with which we have described our process, that our invention is necessarily limited to the specific process described.

Various modifications may be made by those skilled in the art, without departure from our invention. The electrolytic cell may be greatly varied in construction.

What we claim is:—

1. The process of producing aluminum-magnesium alloys, which consists in electrolyzing magnesium oxid dissolved in a fused salt of low specific gravity in the presence of a cathode of molten aluminum-magnesium alloy with which the separated magnesium alloys.
2. The process of producing aluminum-

magnesium alloys, which consists in electrolyzing magnesium oxid dissolved in a fused salt in presence of a cathode of molten aluminum-magnesium alloy with which the separated magnesium alloys.

3. The process of producing aluminum-magnesium alloys, which consists in electrolyzing magnesium oxid dissolved in a fused fluorid in the presence of a cathode of molten aluminum-magnesium alloy with which the separated magnesium alloys.

4. The process of producing aluminum-magnesium alloys, which consists in electrolyzing magnesium oxid dissolved in fused magnesium fluorid and a fluorid of a more electro-positive metal in the presence of a cathode of molten aluminum-magnesium alloy with which the separated magnesium alloys.

5. The process of producing aluminum-magnesium alloys, which consists in electrolyzing a combined fused bath of a magnesium compound and an aluminum compound.

6. The process of producing aluminum-magnesium alloys, which consists in electrolyzing magnesium oxid and aluminum oxide dissolved in a fused fluorid bath.

7. The process of producing aluminum-magnesium alloys, which consists in introducing into a fused bath of magnesium fluorid and a fluorid of a more electro-positive metal, a mixture of magnesium oxid and aluminum oxid, and electrolytically decomposing the same.

8. The process of producing aluminum-magnesium alloys, which consists in introducing into a fused bath of magnesium fluorid and lithium fluorid, a mixture of magnesium oxid and aluminum oxid, and electrolytically decomposing the same.

In witness whereof, we have hereunto signed our names in the presence of two subscribing witnesses.

FRANZ VON KÜGELGEN.  
GEORGE O. SEWARD.

Witnesses:

J. H. WEBB,  
C. OFFERHAUS.